

Sept. 22, 1953

R. J. BALLARD

2,653,266

VAPOR ELECTRIC DEVICE

Filed Sept. 27, 1950



Fig. 1.



Fig. 2.



Fig. 3.

WITNESSES:

*Robert C. Baird*  
*W. B. Groome*

INVENTOR

Robert J. Ballard.

BY *O. B. Buchanan*

ATTORNEY

## UNITED STATES PATENT OFFICE

2,653,266

## VAPOR ELECTRIC DEVICE

Robert J. Ballard, West Newton, Pa., assignor to  
Westinghouse Electric Corporation, East Pitts-  
burgh, Pa., a corporation of Pennsylvania

Application September 27, 1950, Serial No. 187,111

7 Claims. (Cl. 313—212)

1

My invention relates to a vapor electric device and particularly to a device utilizing the vapors of certain alkali metals.

Since the invention of a sealing material which will withstand the chemical activity of the alkali metals, it is now possible to construct power type tubes utilizing the alkali metals such as cesium, rubidium and potassium having an arc drop of the order of 3.8 volts and an overall efficiency of the order of 98%. However, certain drawbacks to the commercial utilization of these devices are still apparent. One of these is the size and weight of the cathode necessary to produce a desirable current output. For example, a cathode capable of delivering a current of the order of 1,000 amperes would have a total surface area of the order of 350 square inches and a total weight, as now constructed, of the order of 36 pounds.

I have discovered that by providing a cathode surface of substantially pure nickel with a small percentage of impurities consisting essentially of phosphides the emission rate of a cesium coated cathode can be increased so that a cathode having an area of 350 square inches is now capable of delivering a current of the order of 2,500 amperes. Also, since the cathode action is apparently only a surface phenomena, it is now possible to construct the cathodes of a cheap metal and to provide a coating of the nickel and nickel phosphide so that the total cost and weight of the cathode can be considerably reduced. For example, the 36 pound cathode of the prior art can be reduced to substantially 32 pounds by utilizing my invention.

Heretofore, the best possible commercially available cathodes for cesium tubes were constructed of substantially pure nickel, but because of the mechanical weakness of nickel, the size and shape of the cathode has been materially circumscribed. However, I have found that the cathode can now be constructed of suitable materials having sufficient strength, such as steel, and the coating of nickel and nickel phosphide applied to the surface of the cathode and still produce a satisfactory emission device far superior to the heretofore known nickel cathodes.

It is accordingly an object of my invention to provide a cesium-vapor-electric device having an increased current capacity.

It is a further object of my invention to provide a cathode having a high emission characteristic per unit of surface area.

It is a further object of my invention to provide a cathode, the active surface of which is

2

composed of nickel with a small percentage of nickel phosphide included.

Other objects and advantages of my invention will be apparent from the following detailed description taken in conjunction with the accompanying drawing, in which:

Figure 1 is an elevation partially in section of a vapor electric device according to my invention;

Fig. 2 is a diagrammatic illustration of the emission characteristics of nickel and nickel phosphide cathodes; and

Fig. 3 is an enlarged section of a portion of the cathode of Fig. 1.

In the exemplary embodiment of my invention, the vapor electric device comprises an anode 10, preferably in the form of a cylindrical container having an opening at one end in which the cathode member 12 is inserted and sealed by means of a glass-metal seal 13 resistant to the action of alkali metal vapor to provide a substantially closed container. The cathode tube 14 is hollow and contains a heating element, the terminals 16 of which extend beyond the cathode 12, as shown. In order to provide sufficient cathode surface area, the cathode 12 is provided with a large number of extensions or fins 17 having a small space between the fins.

In order to prevent excessive transfer of heat from a cathode 12 to the anode 10, a heat shield 18 is normally provided around the cathode 12 and that portion adjacent the enlarged surface area section 17 of the cathode 12 is provided with openings 19 for the passage of the electrons from

the cathode 12 to the anode 10. The anode 10 itself is usually provided with a heat-absorbing inner surface 20 so that the heat which does impinge on the anode 10 is readily absorbed and passed to the coolant which is normally circulated in any desired manner around the outside of the anode 10.

A quantity of cesium is placed in the container to provide the actuating vapor and as is known the cesium deposits in a probably non-atomic layer on all of the metal surfaces in the container.

While the exact action is not surely known, it is known that the layer of cesium on a metal, such as nickel, which has a work function in excess of the ionization potential of cesium vapor, produces a surface of apparent low work function in that it readily emits a large flow of electrons at a relatively low temperature. The improved cathode coating according to the present invention in some manner not fully understood greatly

increases the emission from the cesium-covered surface and also decreases the temperature at which such emission occurs. Not only is the high emission highly desirable, but the reduction in cathode temperature is very important in that it reduces the difficulties in maintaining the associated electrodes below an emitting temperature.

The Bureau of Standards in 1946 developed an improved process of nickel plating by chemical reduction (Research Paper 1835). This process was heretofore supposed to produce substantially pure nickel plating and has an advantage over electroplating in that odd shapes and deep recesses are equally well plated with the smooth exterior surfaces. I have found that nickel plating deposited by this process does indeed contain impurities, mostly in the form of phosphides, particularly nickel phosphide. In a typical example of freshly deposited nickel plating, according to this process, it was found to contain substantially 93% pure nickel with approximately 7% of phosphides. Heat treating reduced the phosphide content to substantially 3%.

The improved cathode 12 is produced by constructing the basic body elements 14 and 17 of any metal having the desired mechanical properties and depositing by chemical reduction a nickel plate 21 on the active surface. As set forth the resultant plate or active surface 21 is composed of about 93% nickel and about 7% impurities mostly in the nature of phosphides. The plate 21 is heat treated at 1100° C. in a non-oxidizing atmosphere for about a half hour when the phosphides are found to be reduced to about 3% of the total plate.

The plate 21 can be deposited from either of the following baths:

|                                   | Basic   | Acid  |
|-----------------------------------|---------|-------|
| Nickel Chloride.....              | 30-40   | 30-40 |
| Sodium Hypophosphite.....         | 10-15   | 10-15 |
| Ammonium Chloride.....            | 50-60   |       |
| Sodium Citrate.....               | 100-110 | 10-15 |
| Ammonium hydroxide to pH of.....  | 8-10    |       |
| Potassium Hydroxide to pH of..... |         | 4-6   |
| Temperature.....pH° C.....        | 90-95   | 90-95 |

I have found that this chemically deposited nickel coating 21, containing the phosphide impurities, has a marked advantage as an electron emitter over the heretofore known electron emitters. For example, as shown by curve 30 in Fig. 2, a pure nickel electrode has a maximum emission of the order of 2.8 amperes per square inch at an electrode temperature of 780° C. with a vapor pressure corresponding to 180° C. Normally, this vapor pressure is controlled by the anode temperature. However, as shown by curve 31 the nickel and phosphide coating 21, according to my process, had a total emission of 6.8 amperes per square inch at a cathode temperature of 700° C. and an anode temperature or vapor pressure temperature of 180° C.

The increase in emission at a lower temperature not only increases the current rating of the tube but materially decreases the operating difficulties in the tube. Since the radiation from any heated surface is substantially at the fourth power of the temperature of the surface, the reduction from 780° C. to 700° C. has materially reduced the radiated energy and makes it much easier to cool the anode or any control electrodes to a safe operating temperature.

Advantage of the increased electron emission can be taken by further reducing the vapor pres-

sure, and consequently the cathode emission temperature. For example, if the vapor pressure temperature is dropped from 180° C. to 160° C., as shown by curve 32, my improved cathode construction provides an emission of approximately 5.8 amperes per square inch at a cathode temperature of 660° C., or in other words, I have been able to get more than double the cathode emission from my improved cathode construction with a reduction of over 120° C. in the emitting surface.

The utilization of the chemically deposited coating 21 as the active cathode surface materially improves the possibilities as to cathode construction. For example, the cathode structure 12 may be made of steel or iron alloy which is easy to fabricate and has inherently great strength even when hot. Also the weight can be somewhat reduced as the density of the iron alloy is less than that of nickel which has heretofore been required.

The improved cathode of the present invention can be utilized either to increase the anode-cathode current per tube, or obviously if the current per tube is to remain constant, a great decrease in the size and weight of the tube will be immediately possible.

While I have shown a preferred embodiment of my invention and described the same according to the best of my present knowledge thereof, I desire it to be understood that such embodiment is exemplary only and that changes and modifications can be made without departing from the spirit of my invention.

I claim as my invention:

1. A vapor electric valve comprising a container, a cathode in insulated relation to said container, a heater maintaining said cathode at emitting temperature, at least the emitting surface of said cathode consisting of nickel containing a small portion of nickel phosphide and a quantity of cesium providing a working vapor in said container and cooperating with said emitting surface to produce high electron emission at low temperature of said surface.

2. A vapor electric valve comprising a container, a cathode in insulated relation to said container, a heater maintaining said cathode at emitting temperature, at least the emitting surface of said cathode consisting of nickel containing 3 to 7 per cent of nickel phosphide and a working vapor in said container cooperating with said emitting surface to produce high electron emission at low temperature of said surface.

3. An electric discharge device comprising an anode, a cathode in spaced insulated relation to said anode, heating means maintaining said cathode at an electron emitting temperature, the surface of said cathode consisting of nickel containing impurities of the order of 3 to 7 per cent, said impurities being essentially nickel phosphide, a quantity of cesium in said device, said cesium cooperating with said cathode surface to produce an emission of the order of 6.5 amperes per square inch of cathode surface at a cathode temperature of 700° C. and an anode temperature of 180° C.

4. In a hot-cathode vapor electric discharge device utilizing a metal vapor, selected from the group comprising cesium, rubidium and potassium, as the ionizable medium, a cathode comprising a metal body, at least one other electrode, and an enclosing housing, characterized by at least the active portion of said cathode body having a surface-coating layer composed of

nickel containing small quantities of phosphides, particularly nickel phosphide.

5. In a hot-cathode vapor electric discharge device utilizing a metal vapor, selected from the group comprising cesium, rubidium and potassium, as the ionizable medium, a cathode comprising a metal body, at least one other electrode, and an enclosing housing, characterized by at least the active portion of said cathode-body having a surface-coating layer composed of nickel containing from 3 to 7 per cent of phosphides, particularly nickel phosphide.

6. In an electric discharge device having a heated cathode in the presence of cesium vapor,

a cathode body constructed of a ferrous metal alloy and an active surface coating layer composed of nickel containing a small percentage of phosphides, particularly nickel phosphide.

5 7. In an electric discharge device having a heated cathode in the presence of cesium vapor, a cathode body constructed of a ferrous metal alloy and an active surface coating layer composed of nickel containing 3 to 7 per cent of phosphides, particularly nickel phosphide.

10 ROBERT J. BALLARD.

No references cited.